

(No Model.)

I. COPELAND.

CEMENT COATED NAIL.

No. 362,940.

Patented May 17, 1887.



FIG. 1.



FIG. 2



FIG. 3.

WITNESSES.

L. R. Churchill  
Warren A. Reed

INVENTOR.

Ira Copeland.

# UNITED STATES PATENT OFFICE.

IRA COPELAND, OF BROCKTON, MASSACHUSETTS.

## CEMENT-COATED NAIL.

SPECIFICATION forming part of Letters Patent No. 362,940, dated May 17, 1887.

Application filed January 19, 1887. Serial No. 224,751. (No model.)

*To all whom it may concern:*

Be it known that I, IRA COPELAND, of Brockton, in the county of Plymouth and State of Massachusetts, have invented a new 5 and useful Improvement in Nails, of which the following is a full, clear, and exact description.

The primary object of this invention is to increase the tenacity or holding power of nails after being driven.

10 The invention consists in coating nails throughout their entire length with certain viscous substances. These substances are so sensitive to heat that the coating of the nail is somewhat softened by the heat produced in 15 the act of driving the nail, and consequently the nail is cemented firmly into its socket when driven.

A secondary object of this invention is found 20 in the preservative effect of the coating, both upon the nail and upon the substance into which the nail may have been driven, especially when used in localities subject to dampness.

Considering both objects to be attained by 25 this improvement, my experience would indicate Trinidad asphalt as one of the best substances available. It may be used in its natural condition or tempered by the addition of paraffine or some non-volatile oil—as, for instance, the residuum from the distillation of 30 petroleum—but there is a wide range of substances susceptible of use for the coating, embracing coal-tar, asphalt, and other bituminous substances, various resins, gums, waxes, and 35 their compounds.

To effectually apply the coating material to the nail, it is necessary to have both the nail and the coating material heated to a temperature at least high enough to melt the coating 40 material.

I find that the wire nail gives much more satisfactory results than the cut nail; but the latter may also be used.

When the nail is driven, the coating material is somewhat displaced from the foremost 45 portion of the nail, and a part of the coating gradually accumulates near the outer portion of the socket in driving, so that when the head is sunk into its socket it is embedded in a layer of coating material. A sufficient amount of 50 coating material remains adhering along the shaft of the nail, gradually increasing in thickness from the point toward the head, to firmly unite the shaft of the nail to the substance into which it is driven.

55 In the drawings, Figure 1 represents a perspective of the nail; Fig. 2, a section of the nail; Fig. 3, a section to show the action of the driven nail.

I am aware that metal-coated nails, or nails 60 coated with any substance which forms an integral part of the nail itself, so that when driven the coating maintains its position relative to the principal substance of the nail, are not new. The coating of my nail is in some 65 degree plastic and is in some degree removed from its original position in being driven.

What I claim, and desire to secure by Letters Patent, is—

A cement-coated nail, substantially as and 70 for the purpose set forth.

In testimony whereof I have signed my name to this specification, in the presence of two subscribing witnesses, this 12th day of January, A. D. 1887.

IRA COPELAND.

Witnesses:

LUCIUS R. CHURCHILL,  
WARREN A. REED.